

## 1

2,926,125

**COATING ARTICLES OF MAGNESIUM OR MAGNESIUM BASE ALLOYS**

Jack Eliwood Cuthbert Currah, Reddendale, Ontario, and Alfred Rudin and Max Morf, Beloeil, Quebec, Canada, assignors to Canadian Industries Limited, Montreal, Quebec, Canada, a corporation of Canada

No Drawing. Application October 22, 1956  
Serial No. 617,287

Claims priority, application Canada March 17, 1956

8 Claims. (Cl. 204—56)

This invention relates to a method of producing coatings of a protective nature on the surface of articles of magnesium or magnesium base alloys. It more particularly relates to an improved method of electrolytically coating the surfaces of articles of magnesium or magnesium base alloys and to the electrolytic bath used in said method.

Magnesium or magnesium base alloys exhibit good resistance to atmospheric corrosion, but are attacked relatively rapidly by most neutral and acidic salt solutions. The corrosion appears to be of the hydrogen-evolution type, i.e., hydrogen is liberated at cathodic areas and magnesium goes into solution from anodic areas. The extent of corrosion depends on the corroding medium, the composition of the alloy and the time of exposure. Magnesium and magnesium base alloys are normally strongly anodic and have a pronounced tendency to dissolve when in electrical contact with other metals in an electrolyte. All commonly used metals will cause galvanic corrosion of magnesium or magnesium base alloys in a conductive solution.

Most paints and varnishes do not adhere well to untreated magnesium or magnesium base alloys because magnesium hydroxide, which is formed as a corrosion product, is strongly alkaline and causes peeling of the paint film. Magnesium and magnesium base alloys are usually protected by painting after a chemical or electrochemical surface treatment.

Several good anodic treatments have been developed recently but none of these treatments has produced a corrosion-resistant coating which does not spall, crack or flake on bending.

It is an object of this invention to provide a method of producing a protective coating upon the surface of articles of magnesium or magnesium base alloys, which coating is an improvement over coatings heretofore available.

A particular object is to provide a method of producing a protective coating upon the surface of articles of magnesium or magnesium base alloys, which coating is uniform in thickness and appearance and resistant to corrosion, and which does not spall on bending or flexing of the article.

A further object is to provide an electrolytic bath for use in such a method.

Other objects of this invention and advantages thereof will appear hereinafter.

Broadly speaking, the aforesaid objects are accomplished by treating electrolytically articles of magnesium or magnesium base alloys in an aqueous solution comprising as essential ingredients an alkali metal borate and a member of the group consisting of hydrogen peroxide, soluble peroxygen compounds and compounds which yield hydrogen peroxide in solution.

It has been found that a protective thin layer of black or grey appearance can be obtained on articles of mag-

## 2

nesium or magnesium base alloys by treating them electrolytically in an aqueous solution comprising as essential ingredients an alkali metal borate and hydrogen peroxide or a compound which yields hydrogen peroxide in solution. The so-produced coating securely adheres to the surfaces to which it is applied, and is very resistant to corrosion.

In treating articles according to the invention, either direct current or alternating current may be used. The 10 coatings produced by the treatment with direct current form more rapidly, effect a more even coverage and exhibit a better appearance than those produced with the aid of alternating current. When alternating current is used, the article is, of course, anodic during a portion 15 of the cycle. The cathode may consist of any suitable material such as magnesium, aluminum, stainless steel, copper, graphite, etc.

Before carrying out the coating process, the articles 20 of magnesium or magnesium base alloys to be coated, are suitably cleaned in conventional manner according to the nature of the foreign matter to be removed. Thus, the removal of oil and grease, and of some of the usual chemical finishes, may be effected by immersing the articles in a hot alkaline stripping solution comprising, for 25 example, caustic soda and diethylene glycol.

It is desirable to activate the surface of the article to be coated with acid as a preliminary step before coating. If an alkaline cleaning step has been used, no significant current can be passed through the coating bath 30 unless the article is given an acid activation. This can be conveniently carried out by dipping the articles in a chromic nitrate pickling solution at room temperature. A momentary dip is sufficient to activate the articles to 35 receive the coating but longer periods of immersion are desirable if the articles are originally fairly dirty.

Ordinary fabricated articles of magnesium or magnesium base alloys which have not received any special treatment may be satisfactorily prepared for the electrolytic treatment of the invention, by conventional mechanical methods.

The electrolytic coating solution of the invention may be fortified with certain other ingredients thereby producing still better coatings. For example, the addition of ingredients such as alkali metal oxalates or dextrin 40 reduces the tendency of the article to become pitted during the anodic treatment.

Borax, sodium metaborate or a mixture of boric acid and sodium hydroxide may be used alone, or in combination, as the source of borate ions. Good coatings are 50 always formed when any one or a combination of these chemicals is present in solution in a concentration equivalent to 0.5 g./l.  $B_2O_3$  or greater. It is preferable to operate with a borate concentration considerably higher than the minimum values in order to obtain a good 55 coating within a shorter application time.

At least a detectable trace of peroxide is required in the electrolyte for coating formation. When larger amounts of peroxide are used, there is a tendency for the anode to become pitted and for the coating to develop a black crust or not to be adherent. This crusting and pitting may be avoided by working at lower current density. While relatively concentrated peroxide solutions may be used it is preferable to use moderate concentrations for economical purposes since higher permissible current densities result in a shorter coating time. The maximum values of the current densities or voltages used are affected by solution composition and degree of agitation of the electrolyte.

The lowest pH at which a satisfactory coating can be 70 formed is about 8.0, but the quality of the coating appears to improve with a higher pH. The upper pH limit is the pH at which the solution precipitates.

Coatings can be formed at a temperature range extending from the freezing point of the solution to about 85° C., depending on the kind of articles to be coated. It is preferable, however, that the coating process takes place at a temperature range extending from 20° C. to 30° C.

The solution used for carrying out the coating treatment according to the invention may be prepared in various ways depending upon the choice of ingredients, and the pH may be adjusted to the desired limit by the addition to the solution, if necessary, of an alkali such as sodium hydroxide.

Conventional magnesium racks and clamps may be employed for carrying out the electrolytic process. It is essential that the racks or clamps make good contact with the articles to be coated, since the coating acts as an insulator. A brief dip in dilute nitric acid or fluoride-containing solutions inhibits them from being coated and therefore keeps them clean. This feature is an advantage since no current need be lost in coating them.

The following table sets forth examples of preferred operating baths for the production of coatings according to the invention.

7. A method as claimed in claim 2 wherein a temperature range extending from the freezing point of the solution to about 85° C. is maintained during the entire coating time.

8. A method as claimed in claim 2 wherein a temperature range extending from 20° C. to 30° C. is maintained during the entire coating time. 5

## References Cited in the file of this patent

## UNITED STATES PATENTS

2,206,028 Buzzard ----- July 2, 1940  
2,276,353 Thompson ----- Mar. 17, 1942

## FOREIGN PATENTS

815,155 France ----- July 7, 1937